

Patented June 5, 1923.

## UNITED STATES PATENT OFFICE.

WILLIAM ALBERT RUDDELL, OF ASBURY PARK, NEW JERSEY.

## METAL POLISH.

Application filed December 28, 1921. Serial No. 525,446.

No Drawing.

To all whom it may concern:

Be it known that I, WILLIAM A. RUDDELL, a citizen of the United States, residing at Asbury Park, in the county of Monmouth and State of New Jersey, have invented 5 certain new and useful Improvements in Metal Polish, of which the following is a specification.

This invention relates to metal polishing 10 compositions and has as its object to provide a composition especially useful in polishing silverware, tinware, aluminum, copper, brass, and other metals in cash registers, typewriters, automobile parts, etc.

Another object of the invention is to provide a polishing composition which will clean, polish, and plate the surface to which it is applied and which composition may be employed to obtain a smooth finish and a 20 high polish without the expenditure of great energy.

Another object of the invention is to provide a polishing composition which will not freeze in cold weather and which will keep 25 indefinitely.

The composition embodying the invention consists of a mixture of silver cyanide, potassium nitrate, potassium cyanide, salt, white borax, whiting and alcohol. The 30 portions in which these ingredients are present in the compositions may vary but ordinarily the composition will contain the ingredients in the following proportions:

Silver cyanide about 1 oz., potassium nitrate about 1 oz., potassium cyanide about 35 8 ozs., white borax 1 to 2 tablespoonfuls, whiting 2 lbs., salt, 1 to 4 tablespoonfuls, distilled water about 2 qts., alcohol (grain, wood, or denatured) from 10 to 50 per cent.

40 The amount of alcohol employed will, of

course, vary with climatic conditions, more alcohol being employed where the composition is to be used in cold weather, or in a cold climate.

In preparing the polishing compositions 45 I preferably proceed as follows: In a portion of the water I dissolve approximately eight ounces of potassium cyanide and in the remainder of the water I dissolve approximately one ounce of silver nitrate. 50 These two solutions are then mixed and in accordance with the chemical reaction which takes place the silver content is converted into silver potassium cyanide, so that the resulting mixture is a solution of silver-potassium cyanide, potassium cyanide and potassium nitrate. To this mixture the whiting and alcohol, salt, and borax are then added and the whole is thoroughly stirred 55 for about fifteen minutes. The composition is then ready for use and after a small quantity thereof has been poured upon the surface to be polished the surface is wiped or rubbed with a soft cloth preferably 60 dipped in warm water, after which the surface is polished with a dry soft cloth.

Instead of employing potassium cyanide, I may, of course, make use of sodium cyanide.

Having thus described the invention, 70 what I claim as new is:

A polishing composition comprising a mixture of silver-potassium cyanide, potassium cyanide, potassium nitrate, borax, 75 whiting, water and alcohol, in the proportions resulting from the ingredients named in the quantities herein specified.

In testimony whereof I affix my signature.

WILLIAM ALBERT RUDDELL. [I. S.]